

2,133,433

Oct. 18, 1938.

L. S. DEITZ, JR.  
PURIFICATION OF LEAD  
Filed Nov. 27, 1936

FIG. 1



FIG. 3



FIG. 2



INVENTOR  
L. S. DEITZ JR.

*L. S. Deitz Jr.*  
ATTORNEY

## UNITED STATES PATENT OFFICE

2,133,433

## PURIFICATION OF LEAD

Louis Scott Deitz, Jr., Metuchen, N. J., assignor to  
 Western Electric Company, Incorporated, New  
 York, N. Y., a corporation of New York

Application November 27, 1936, Serial No. 113,036

4 Claims. (Cl. 75—78)

This invention relates to the purification of lead, and more particularly to methods of and apparatus for removing such impurities as zinc, arsenic, tin and antimony from lead and lead alloys.

It is well known that zinc, arsenic, tin and antimony may be removed from molten lead by oxidizing these impurities with solid oxidizing agents, such as sodium nitrate, in the presence of an alkali hydroxide, such as sodium hydroxide, or other fluxes. However, if the addition of the oxidizing agent and the intermingling of the lead and the reagents are not properly controlled, the process will require a long time for completion, or will result in the oxidation of large quantities of the lead along with the impurities, or else will require the use of excessive amounts of reagents.

It has been suggested heretofore that molten sodium hydroxide, or a mixture thereof with sodium chloride, might be employed in contact with a bath of molten impure lead, and that sodium nitrate might be added gradually at a constant rate to the molten flux, and thereby indirectly to the lead. However, if the quantity of the nitrate added at any time in the processes formerly employed was small enough to prevent oxidation of large quantities of lead near the end of the process, the process required a long time to reach completion. Furthermore, if the impure lead and the purifying reagents were not brought into intimate contact or these materials were intermingled slowly, the process was inefficient because of loss of oxygen through the escape of decomposition products of the nitrate. In addition, if the whole lead bath was not effectively brought into the reaction by proper agitation or circulation, some of the lead was permanently oxidized instead of the impurities which normally oxidize more readily than the lead.

Among the objects of the present invention is the provision of simple, efficient and rapid methods of removing impurities from lead and lead alloys, either selectively or in bulk.

Another object of the invention is the provision of simple and efficient apparatus for practicing the purification methods embodying the invention.

In accordance with one embodiment of the invention, lead is purified by rapidly bringing successive portions of a body of molten impure lead

into intimate contact with a molten alkali hydroxide and by adding an oxidizing agent thereto at a gradually decreasing rate. These materials are thoroughly and rapidly brought into reactive contact with each other by means of an agitator provided with a plurality of projecting pins which pass through the floating layer of hydroxide and oxidizer and also through a portion of the molten lead.

The above described and other objects and features of the invention will be apparent from the following detailed description of specific embodiments thereof and the annexed drawing, in which

Fig. 1 is a vertical section of a lead purifying apparatus embodying the invention,

Fig. 2 is a perspective view of an agitator forming a part of the lead purifying apparatus, and

Fig. 3 is a graph showing curves plotted from data pertinent to the practice of a process embodying the invention.

In accordance with the invention, impurities such as zinc, arsenic, tin and antimony may be removed from lead, either selectively or in bulk, by placing a charge 10 of the lead within a kettle 11, which is heated to a temperature well above the melting point of lead by any suitable means (not shown), such as an oil burner. The lead may be introduced into the kettle in the molten state or it may be melted therein, as desired. The dross which accumulates upon the surface of the molten lead is skimmed off and an alkali hydroxide is introduced upon the surface of the molten lead and forms a layer 12 of molten hydroxide thereon. The amount of the hydroxide introduced is determined by and is proportional to the quantity of a particular impurity or impurities which it is desired to remove from the lead.

The kettle 10 is provided with an agitator indicated generally by the numeral 14, which comprises a horizontal circular plate 15 having a circular series of pins 16—16 which extend upwardly from the plate 15. The plate 15 is rigidly mounted upon a shaft 18 supported by a bearing member 19 and the shaft is provided at its upper extremity with a gear 20 meshing with a gear 21 secured upon a shaft 22 which is connected to any suitable source of power (not shown), such as an electric motor. The agitator 14 is so positioned within the kettle 10 and the

parts of the agitator are so proportioned that the plate 15 is below the surface of the molten lead and the pins 16-16 extend upwardly through a portion of the molten lead and entirely 5 through the layer of molten hydroxide upon the surface of the lead.

After the layer of molten hydroxide has been introduced, the agitator 14 is placed into operation and a solid oxidizing agent, such as sodium 10 nitrate, is added to the bath at a gradually decreasing rate and in such a manner that the quantity of oxidizing agent added at any time is proportional to the amount of the impurity being removed that is present at that time in the 15 bath or molten lead. The impurities in the lead are oxidized by the nitrate or other oxidizing agent and the oxidized impurities are absorbed by the layer of molten hydroxide and are thus removed from the metal. The agitator 14 keeps the 20 nitrate stirred into the layer of hydroxide and also keeps the hydroxide in motion. It also rapidly brings particles of the molten lead into intimate contact with the hydroxide thus insuring a substantially complete reaction between the 25 nitrate carried by the hydroxide and the molten lead.

This operation is continued until all of the oxidizing agent necessary to remove the impurity in question has been added and has had sufficient 30 time to react with the lead, whereupon the agitator is stopped and the hydroxide slag is skimmed off of the molten lead by means of a perforated shovel or other suitable means. The purified lead may then be removed from the kettle 35 and cast into pigs or used directly for any purposes for which the purified lead is intended.

If there is only one impurity, such as tin, in the lead or if there is no need to separate the slags obtained by removing several impurities or to remove 40 certain impurities and leave others in the lead, then the quantity of hydroxide employed and the total amount of oxidizing agent used are proportional to the total quantity of impurities present in the lead. However, it may be desirable 45 to remove only one of two or more impurities from the lead, or it may be advantageous to remove the various impurities successively and to collect the slags produced by the removal of each impurity separately. In this event the purification 50 is effected in steps, in each of which a sufficient quantity of hydroxide is used and enough oxidizing agent is gradually added at a constantly reducing rate to remove only a particular impurity. When the removal of this particular impurity is completed 55 the agitator is stopped and the hydroxide slag withdrawn. These operations may be repeated if desired for the removal of another impurity, making certain that the hydroxide and oxidizer added are employed in the quantities requisite for the removal of this impurity. This operation may be repeated for as many times as may be necessary or desirable to purify the lead to the desired extent. It has been found that the usual impurities in lead, such as zinc, arsenic, tin 60 and antimony, are removed by this process in this sequence.

Specific examples of the removal of various impurities in accordance with the invention are as follows:

70 *Example 1.*—A ten pound lot of a lead-tin alloy containing about 3% tin may be purified to the point where it contains only about .02% tin by covering the molten alloy with nine-tenths of a pound of sodium hydroxide, i. e. three parts of 75 sodium hydroxide per part of tin in the lead, and

adding sixty-six grams of sodium nitrate thereto at a constantly decreasing rate, the amount added at any particular time depending upon the quantity of tin present in the lead at that time. The rate of addition of the sodium nitrate and the results obtained are indicated in the following table:

| Period          | NaNO <sub>3</sub><br>added | At end of period          |                              |                             | 10 |
|-----------------|----------------------------|---------------------------|------------------------------|-----------------------------|----|
|                 |                            | Percent<br>Sn in<br>alloy | Total<br>lbs. tin<br>removed | Percent<br>tin re-<br>moved |    |
| 1st 15 minutes  | 14 1/2                     | 2.3                       | .07                          | .23                         | 15 |
| 2nd 15 minutes  | 12                         | 1.8                       | .12                          | .40                         |    |
| 3rd 15 minutes  | 10                         | 1.3                       | .17                          | .60                         |    |
| 4th 15 minutes  | 8                          | 1.0                       | .20                          | .73                         |    |
| 5th 15 minutes  | 6 1/2                      | 0.7                       | .23                          | .83                         |    |
| 6th 15 minutes  | 5                          | 0.5                       | .25                          | .90                         |    |
| 7th 15 minutes  | 4                          | 0.3                       | .27                          | .93                         | 20 |
| 8th 15 minutes  | 3                          | 0.1                       | .29                          | .97                         |    |
| 9th 15 minutes  | 2                          | 0.03                      | .297                         | .99                         |    |
| 10th 15 minutes | 1                          | 0.02                      | .298                         | .99.3                       |    |
| 2 1/4 hours     | 66                         |                           |                              |                             |    |

Example 2.—Ten pounds of another lead alloy 25 containing about 1% antimony and .07% tin may be detinned by covering the molten metal with sodium hydroxide and adding 2 1/2 grams of sodium nitrate thereto at a gradually decreasing rate over a period of about thirty minutes. At the end of this period the agitator should be stopped and the slag withdrawn. The lead will then contain about .9% antimony and less than .02% tin.

Example 3.—Another lead alloy containing .9% 35 antimony and .04% tin may be purified as follows:

Ten and a half pounds of the alloy may be melted and covered with a quantity of sodium hydroxide equivalent to at least three times the amount of the total antimony and tin therein, the agitator started and sodium nitrate added to the molten material at the following rate:

| Period         | NaNO <sub>3</sub><br>added | Grams |
|----------------|----------------------------|-------|
| 1st 15 minutes |                            | 9.0   |
| 2nd 15 minutes |                            | 6.5   |
| 3rd 15 minutes |                            | 4.0   |
| 4th 15 minutes |                            | 2.5   |
| 5th 15 minutes |                            | 1.5   |
| 6th 15 minutes |                            | 0.5   |

After this treatment the slag should be withdrawn and the metal will contain less than .02% antimony and less than .02% tin.

In all of these examples, the lead is purified without the oxidation of excessive quantities of lead along with the impurities. Also the purification is accomplished at a much more rapid rate 60 than was possible by the use of methods and apparatus heretofore known and requires a smaller quantity of oxidizing agent than was required by former methods. This is due to the fact that when large quantities of impurities, such as tin and antimony, are present in lead, they may be much more rapidly oxidized than may relatively small quantities of these materials without oxidizing excessive quantities of the lead at the same time. Consequently, in accordance with this invention, relatively large quantities of oxidizing agent are added during the initial stages of the purification process and the quantity of oxidizing agent is gradually decreased as the process progresses so that at no stage is there an appreciable 70 75 80 85 90 95

excess of oxidizing agent, but at the same time there is present a sufficient amount of oxidizing agent to react with the impurities at substantially the maximum rate possible for the quantity of impurities then present.

The quantity of oxidizing agent to be added during any given period of the process may be determined by ascertaining the greatest amount of oxidizing agent that can be added to the lead over a fifteen minute period for a given percentage of impurity in the alloy without oxidizing excessive quantities of the lead along with the impurity and without losing the oxidizing power of the nitrate by the escape of excessive amounts of oxidizing gases from the hydroxide. This information may be obtained for a series of lead alloys of different compositions and the results plotted to obtain graphs which may be utilized to practice the invention effectively.

For instance, in purifying the lead-tin alloy of Example 1 above, the maximum quantities of sodium nitrate that could be added in a particular apparatus to a series of lead alloys containing from about 3% tin down to substantially no tin were determined. These values also represent the rate at which sodium nitrate should be added to a lead-tin alloy containing about 3% tin to remove substantially all of the tin therefrom in the most effective manner and are those found in the first column of the table given in Example 1. The summations of these respective values when plotted as a function of time give a curve such as the one designated "A" in the graph shown in Fig. 2 of the drawing. In this graph the ordinates represent the total quantities in grams of sodium nitrate added up to the ends of the respective fifteen minute periods to the lead-tin alloy, while the abscissas for curve "A" represent time in hours. By similar computations, the rate of addition of the oxidizing agent for the removal of other impurities, such as zinc, arsenic and antimony, from lead and lead alloys may be obtained.

If the values from the above graph for the total amounts of sodium nitrate added up to the ends of the respective periods are plotted as a function of the quantity of tin remaining in the lead at the ends of these periods, a line such as "B" in the chart shown on the drawing is obtained. Since the line "B" is a straight line, it is obvious that the quantity of nitrate added at any stage of the operation is directly proportional to the quantity of tin then in the lead.

Theoretically, the best results will be obtained if the oxidizing agent is added to the reaction kettle at a rate that is continually decreasing throughout the operation of the process and in large scale operations it would be feasible to provide an automatic feeder to supply the oxidizing agent in accordance with a predetermined optimum decreasing rate. However, it has been found satisfactory in actual practice to feed to the kettle the amount of oxidizing agent required for any given fifteen minute period at a substantially uniform rate throughout that period.

While sodium nitrate has been described as the oxidizing agent employed in the specific examples given herein, other solid oxidizing agents may be employed with satisfactory results. For example, potassium nitrate, sodium or potassium nitrite, sodium or potassium chlorate, sodium or potassium peroxide, and other similar solid oxidizing agents may be substituted for the sodium nitrate.

The amount of alkali hydroxide employed as a flux should be at least three times as great as

the quantity of impurity which is to be removed from the lead. Instead of the sodium hydroxide employed in the specific example disclosed, potassium hydroxide may be used. Also a part of the sodium or potassium hydroxide may be replaced by sodium chloride, or common salt, if desired.

The slag produced in the purification process is preferably treated in any suitable manner to remove from the excess of alkali hydroxide there- in the products obtained by the oxidizing reaction and to revivify the hydroxide present in chemical combination with these oxidation products. The alkali hydroxide thus recovered from the slag may then be used again in the purification process.

The agitator employed in practicing the processes embodying the invention very effectively mingles the impure lead with the purifying agents and rapidly brings fresh particles of lead into intimate contact with these agents. It also keeps the slag broken up and agitates it thoroughly. As a result, fresh particles of lead and of the refining agents are constantly being rapidly and intimately intermingled and the impurities in the lead are speedily oxidized and removed. While the agitator has been disclosed with the plate which supports the pins immersed in the lead bath with the pins extending upwardly through the slag, the plate may be inverted so that it is above the contents of the kettle and the pins extend downwardly through the slag and into the upper portion of the lead. The plate may also be provided with openings, if desired, to reduce the mass thereof.

What is claimed is:

1. The method of removing oxidizable impurities from molten lead which comprises adding an alkali hydroxide fluxing material, oxidizing the impurities in the lead by adding an oxidizing agent from the group of sodium or potassium nitrate, sodium or potassium nitrite, sodium or potassium chlorate, in successive amounts, each successive amount being less than the preceding amount accordingly as the impurities decrease and each amount being substantially the maximum possible to be added at the time of addition without effecting oxidation of the lead to any substantial extent, and agitating the lead as the oxidizing agent is added.

2. The method of removing the impurities, zinc, arsenic, tin and antimony, or any of them, from lead, which comprises oxidizing said impurities in the presence of an alkali hydroxide by adding a solid oxidizing agent at a gradually decreasing rate, to molten lead containing them and agitating the molten lead, the oxidizing agent being added in successive amounts, each amount so added being substantially the maximum possible to be added at the time of addition without effecting oxidation of lead to any substantial extent, and the successive added amounts diminishing in constant ratio to the diminishing amounts of impurity to be removed present at the successive times of addition.

3. The method of removing oxidizable impurities from molten lead which comprises adding an alkali hydroxide to the lead, oxidizing the impurities in the lead by adding a solid alkali oxidizing compound in successive amounts, each successive amount being less than the preceding amount as the impurities decrease and each amount being substantially the maximum possible to be added at the time of addition without effecting oxidation of the lead to any substantial

extent, and agitating the lead during the addition of the oxidizing compound.

4. The method of removing oxidizable impurities from molten lead which comprises adding sodium hydroxide to the lead, oxidizing the impurities in the lead by adding sodium nitrate in successive amounts, each successive amount being

less than the preceding amount as the impurities decrease and each amount being substantially the maximum possible to be added at the time of addition without effecting oxidation of the lead to any substantial extent, and agitating the lead during the addition of the sodium nitrate.

LOUIS SCOTT DEITZ, JR.